

Feb. 20, 1923.

1,446,332.

J. W. BRAMWELL.

ALLOY AND METHOD OF MAKING SAME.

FILED NOV. 13, 1919.



Inventor—  
Joseph W. Bramwell.  
by his Attorneys—  
Howson & Howson

## UNITED STATES PATENT OFFICE.

JOSEPH WM. BRAMWELL, OF BERWYN, PENNSYLVANIA, ASSIGNOR TO AMERICAN BRONZE CORPORATION, OF BERWYN, PENNSYLVANIA, A CORPORATION OF PENNSYLVANIA.

## ALLOY AND METHOD OF MAKING SAME.

Application filed November 13, 1919. Serial No. 337,778.

*To all whom it may concern:*

Be it known that I, JOSEPH W. BRAMWELL, a citizen of the United States, residing in Berwyn, Chester County, Pennsylvania, have invented Alloys and Methods of Making Same, of which the following is a specification.

One object of my invention is to provide a high grade bearing bronze in rod or tubular form, for use particularly in automatic screw machines for the economical production of bushings of various sizes and lengths, or in sheet form for the economical production by stamping of discs and washers.

Another object of the invention is to provide a method for treating alloys of the above noted class, whereby the valuable qualities inherent in what may be referred to as the raw material are preserved in the improved product, so that for example, an alloy of a certain composition particularly adapting it for use as a bearing metal, when subjected to my method of treatment not only has no impairment of its qualities as a bearing metal but in addition has given to it other qualities adding materially to its value as a material for the manufacture of machine elements or parts;—the invention especially contemplating such a method of procedure in the production of certain articles such as tubular bearings as will materially reduce their cost both in material and labor.

In carrying out my invention I may use apparatus such as is shown in the accompanying drawings, in which—

The figure is a diagrammatic representation in vertical section of a furnace, tank and rolling mill constituting apparatus which may be employed in connection with my invention.

I have discovered that by employing certain methods hereinafter described, I am able to successfully roll, draw or swage a non-ferrous alloy containing more than 85% copper, more than 9½% tin and more than 2% zinc and preferably containing 86½% copper, 11% tin and 2½% zinc. The basic ternary alloy whose low limits are referred to as containing more than 85% of copper, more than 9½% of tin, and more than 2% of zinc, can, within the scope of my process, my claims, and my practice be made to include relatively small additions not to ex-

ceed 2% each of each or several of the metals comprised in the groups or families represented by: aluminum, arsenic, boron, cobalt, magnesium, manganese, molybdenum, nickel, phosphorus, potassium, silicon, titanium, tungsten, uranium, vanadium, zirconium.

In carrying out my invention I heat an alloy of approximately the composition above specified to a temperature of from 932° F. at which the eutectic fuses to 1483° F. and preferably to 1250° F., in a furnace such as is indicated at 1 for a period of time (depending upon the size and mass of the piece under-going manipulation) sufficient to enable such specimen to become thoroughly heated throughout to a temperature within the prescribed limits and then immediately subject the piece to treatment in a suitable cooling medium, preferably by plunging it into a bath 2 of cold water. The specimen is thereafter submitted without further heating, to a rolling, drawing or swaging process in a suitable rolling mill 3 at a speed not in excess of 15 feet per minute, simultaneously with a draft not in excess of .0625", and this process is repeated as occasion requires depending upon the size and mass of the piece undergoing manipulation and upon the ultimate dimensions required. As a result of this treatment the alloy analyzing as above described can be successfully produced in rods, sheets and tubes of dimensions to meet existing and future demands.

In the preparation of rolling equipment for the production of rods and tubes from the alloy as described above, I have discovered the necessity of departure from well-known and commonly used designs of such equipment, for if the grooves in such rolls be concentric, a "fin" will be produced on the specimen which will render it useless. If on the other hand the grooves be "opened" as is the common practice in the rolling of steel and other alloys, such opening will permit the specimen to fracture.

I have discovered that a chamfer or radius between the rolls 4 and 5 of from  $\frac{1}{16}$ " to  $\frac{3}{16}$ " (depending upon the size of the specimen) will obviate this difficulty.

I have further found that in the rolling process a certain fixed relation should exist between the speed of rolls and the amount

of reduction or "draft" of the material possessing the high tin content. For example, at a roll speed of 15 feet per minute, the maximum safe reduction or "draft" was found to be  $\frac{1}{16}$ ", and any greater draft at the same speed caused the material to disintegrate. In accordance with this feature of my invention if

R=reduction or "draft" at each pass—  
10 maximum for any increased speed— $\frac{1}{16}$ ;

S=speed ft. per min. at each pass;

$S_1$ =any other increased speed;

$R_1$ =the "draft" for any other increased speed will be inversely as the fourth powers  
15 of S and  $S_1$ ; then

$$R_1 = \frac{S^4 \times 0.0625}{S_1^4}$$

As a result of my method of treatment the 20 physical properties of an alloy of the chemical composition above noted and having as originally cast an ultimate strength of approximately 45,000 pounds per square inch, a yield point of approximately 22,500 pounds  
25 per square inch, an elongation in 2" of from 9% to 12% and a Brinell hardness number of about 90, can be improved so that the ultimate strength will be over 110,000 pounds per square inch, the elastic limit will be over 30 100,000 pounds per square inch, the elongation over 40% in two inches and the Brinell hardness number over 200.

Also the ductility of the alloy can be materially increased and the specific gravity

increased from 8.66 to 9.01. In short, the 35 wear resisting qualities and consequent desirability and adaptability of the metal as a bearing material are greatly enhanced.

I claim:

1. The method which consists in heating 40 a bronze alloy, containing more than 85% of copper, more than 9 $\frac{1}{2}$ % of tin and more than 2% of zinc, to a temperature of from 932° F. to 1483° F., immediately quenching said alloy in a cooling medium and thereafter compacting the alloy as by rolling, drawing, or swaging.

2. The method which consists in heating 45 a bronze alloy containing more than 85% of copper, more than 9 $\frac{1}{2}$ % of tin and more than 2% of zinc to a temperature below that at which it disintegrates and above that at which the eutectic fuses; and subjecting said alloy to a compacting operation at the speed and draft represented by the formula:— 50

$$R_1 = \frac{S^4 \times 0.0625}{S_1^4}$$

3. The method which consists in heating 55 an alloy containing more than 85% of copper, more than 9 $\frac{1}{2}$ % of tin and more than 2% of zinc to a temperature of from 932° F. to 1483° F. and subjecting said alloy to a compacting operation between rolls having a chamfer or radius of one sixty-fourth 60 of an inch to three-sixteenths of an inch on the edges of their grooves.

JOSEPH WM. BRAMWELL.